

April 2, 1957

J. E. STARECK ET AL

2,787,588

CHROMIUM PLATING

Filed Aug. 12, 1954



2,787,588

## CHROMIUM PLATING

Jesse E. Stareck, Royal Oak, and Ronald Dow, Detroit, Mich., assignors, by mesne assignments, to Metal & Thermit Corporation, New York, N. Y., a corporation of New Jersey

Application August 12, 1954, Serial No. 449,378

7 Claims. (Cl. 204—51)

This invention relates to chromium plating using a 15 chromic acid plating bath and particularly to a method for producing crack-free deposits of chromium.

In co-pending application Serial No. 356,188, filed May 20, 1953, now Patent 2,686,756, issued August 17, 1954, of which the present application is a continuation-in-part, there is described and claimed a method of producing crack-free chromium plate by maintaining, over a range of chromic acid concentration, particular and well defined amounts of catalyst acid radicals whose concentrations are not only self-regulated but also controlled by means of non-catalytic suppressor compounds, and by maintaining the temperature of the bath solution above a particular minimum value.

The present invention has the same purpose as the said copending application and utilizes similar means for accomplishing the purpose except that only a portion of the catalyst acid radical content of the bath solution is controlled by non-catalytic suppressor compounds. In the present method the bath solution comprises chromic acid, two catalyst-supplying compounds, namely, strontium sulfate and an alkali metal silicofluoride, each having a limited solubility in the chromic acid bath, and a soluble non-catalytic alkali metal compound. The alkali metal of the non-catalytic compound is the same as that of the silicofluoride compound and is selected from the group consisting of potassium and sodium. The non-catalytic compound has the effect of controlling the concentration of the dissolved silicofluoride radical in the bath by decreasing the solubility of the alkali metal silicofluoride. The concentrations of the dissolved sulfate and silicofluoride radicals are self-regulated, but the sulfate concentration is not controlled by a non-catalytic compound. Specific non-catalytic compounds are potassium or sodium hydroxide, potassium or sodium bichromate, potassium or sodium carbonate, and potassium or sodium chromate.

The concentration of the chromic acid, expressed as  $\text{CrO}_3$ , in the bath is about 300 to 900 g./l. The amount of the strontium sulfate and the alkali metal silicofluoride, is, in each case, sufficient to saturate the bath with dissolved sulfate and silicofluoride and to provide an insoluble residue of each salt in the bath. The soluble non-catalytic alkali metal compound is present in an amount sufficient to adjust or suppress the concentration of the alkali metal silicofluoride in solution in the bath from the unsuppressed saturation concentration of the latter to a lower concentration such that the sum of the dissolved sulfate ( $\text{SO}_4^{=}$ ) and silicofluoride ( $\text{SiF}_6^{=}$ ) is 2.5 to 10.5 g./l. The concentration of dissolved sulfate is the unsuppressed saturation concentration and may vary from 1.5 to 5.5 g./l., and that of dissolved silicofluoride is the suppressed saturation concentration and may vary from 1.0 to 9.0 g./l., with the sum of the two catalysts lying in the range of 2.5 to 10.5 g./l. The sum of the dissolved sulfate and silicofluoride required varies with the dissolved  $\text{CrO}_3$  in the manner defined by the area ABCD of the graph shown in the accompanying drawing. As noted in the drawing, the graph shows the variation of the chromic

acid concentration in grams per liter with the concentration, in grams per liter, of the sum of dissolved sulfate and silicofluoride. As the chromic acid varies from 300 to 900 g./l., the required catalyst content varies from a low of 2.5 g./l. to a high of 10.5 g./l. Within the area ABCD, the plate that is deposited is crack-free and has the other advantages described hereinafter. At catalyst concentrations that lie above the curve DC, the plate is cracked, and at catalyst concentrations below the curve AB, the plate is nodular and unsuitable. The above-described variation of the chromic acid with the sum of the sulfate and silicofluoride may also be shown by Table 1, which also shows how the sulfate and silicofluoride concentrations may individually vary:

TABLE 1

| $\text{CrO}_3$ ,<br>g./l. | $\text{SO}_4^{=}$ + $\text{SiF}_6^{=}$ ,<br>g./l. | $\text{SO}_4$ , g./l. | $\text{SiF}_6$ , g./l. |
|---------------------------|---------------------------------------------------|-----------------------|------------------------|
| 300                       | 2.5                                               | 1.5                   | 1.0                    |
| 400                       | 2.5-3.0                                           | 1.5-2.2               | 1.0-2.4                |
| 500                       | 3.0-5.2                                           | 1.5-2.8               | 1.0-3.7                |
| 600                       | 3.5-6.5                                           | 1.5-3.5               | 1.0-5.0                |
| 700                       | 4.0-7.8                                           | 1.5-4.2               | 1.0-6.3                |
| 800                       | 4.5-9.2                                           | 1.5-4.8               | 1.0-7.7                |
| 900                       | 5.0-10.5                                          | 1.5-5.5               | 1.0-9.0                |

Preferably, the amount of the non-catalytic alkali metal compound is such as to suppress the concentration of the silicofluoride in solution in the bath from the unsuppressed saturation concentration of the latter to a lower concentration such that the sum of the dissolved sulfate ( $\text{SO}_4^{=}$ ) and silicofluoride ( $\text{SiF}_6^{=}$ ) is 3.0 to 8.5 g./l. The preferred concentration of dissolved sulfate may vary from 1.8 to 5.0 g./l. and that of dissolved silicofluoride from 1.2 to 7.0 g./l., with the preferred sum of the two catalysts lying in the range of 3.0 to 8.5 g./l. and the  $\text{CrO}_3$  varying from 400 to 900 g./l. This referred variation of the sum of the dissolved catalyst radicals with  $\text{CrO}_3$  concentration is as defined by the area JKLM of the graph, and is also set forth in Table 2:

TABLE 2

| $\text{CrO}_3$ | $\text{SO}_4^{=}$ + $\text{SiF}_6^{=}$ | $\text{SO}_4$ | $\text{SiF}_6$ |
|----------------|----------------------------------------|---------------|----------------|
| 400            | 3.0-3.5                                | 1.8           | 1.2-2.0        |
| 500            | 3.5-4.5                                | 1.8-2.2       | 2.0-3.0        |
| 600            | 4.0-5.5                                | 1.8-2.8       | 2.0-4.0        |
| 700            | 4.5-6.5                                | 1.8-3.5       | 2.0-5.0        |
| 800            | 5.0-7.5                                | 1.8-4.2       | 2.0-6.0        |
| 900            | 5.5-8.5                                | 1.8-5.0       | 2.0-7.0        |

A more preferred range of  $\text{CrO}_3$  concentration is 500 to 700 g./l., with the dissolved sulfate varying from 1.8 to 3.5 g./l., the dissolved silicofluoride varying from 2.0 to 5.0 g./l., and the sum of the two catalysts varying from 3.5 to 6.5 g./l.

The chromic acid content may be supplied by adding chromic acid as such to the bath, although a portion may be supplied by the  $\text{CrO}_3$  content of non-catalytic compounds like potassium or sodium bichromate and potassium or sodium chromate. It will be understood that in referring to the bath chromic acid content, it is intended to include, unless specified otherwise, the  $\text{CrO}_3$  added per se, and any  $\text{CrO}_3$  added in the form of one of the foregoing non-catalytic compounds.

The plating bath may be made up by adding a mixture of the solid ingredients, in powdered or granular form, to water and stirring until equilibrium is obtained. The bath may also be maintained in this way.

The plating method comprises passing current in the range of 0.5 to 8, preferably 1 to 3, amperes per square inch (a. s. i.) from an anode to an article cathode im-

mersed in the bath. The bath is operated at a minimum temperature of 140° F., it having been found that below this temperature the plate that is produced is cracked. The upper temperature may extend to the boiling point of the bath but preferably is about 180° F. A preferred temperature range is 145 to 160° F. Generally, with higher temperatures the concentrations of dissolved CrO<sub>3</sub>, sulfate and silicofluoride should be higher, and higher current densities are used.

The crack-free quality of the chromium plate produced by the present method is not only determinable visually but also by means of other tests, as described in the said copending application. The crack-free plate of the invention is also characterized by having a hardness of about 425 to about 825, usually 550 to 700, Knoop. The plate is relatively soft and ductile as compared with conventional chromium plate. It has a smooth texture, a satiny finish, and a dull, matte, white color. It is easy to polish or buff.

The invention may be illustrated by the following examples:

*Example 1*

Using a mixture of 83.5% chromic acid, 13.3% potassium dichromate, 1.0% potassium silicofluoride, and 2.2% strontium sulfate, weight basis, a solution was made up comprising 676 grams of the foregoing mixture per liter of solution. The solution contained 625 g./l. of dissolved CrO<sub>3</sub>, 2.6 g./l. of dissolved sulfate, and 1.6 g./l. of dissolved silicofluoride. A steel rod 3" long x 3/8" diameter, was plated in this solution at 150° F. and 3 a. s. i. for 3 hours, a crack-free plate being produced.

*Example 2*

From a mixture of 410 parts of chromic acid, 284 parts of sodium dichromate, 14.3 parts of sodium silicofluoride, and 7.2 parts of strontium sulfate, all parts by weight, an aqueous solution was made up analyzing as follows: 601 g./l. CrO<sub>3</sub>, 2.2 g./l. sulfate, and 1.8 g./l. silicofluoride. A steel mandrel of conventional size was plated in this solution for 0.5 hour at 2.5 a. s. i. and 150° F. A dull, white crack-free deposit of chromium of 0.3 mil thickness was produced on the mandrel.

*Example 3*

A mixture of 446 parts of chromic acid, 80 parts of potassium dichromate, 10 parts of potassium of silicofluoride, and 10 parts of strontium sulfate, all parts by weight, were dissolved in water to form a solution containing 500 g./l. of dissolved CrO<sub>3</sub>, 1.8 g./l. of sulfate, and 2.0 g./l. of silicofluoride. A steel mandrel of conventional size was plated in this solution at 150° F. and 3 a. s. i. for 1 hour, a smooth, dull white crack-free plate being produced.

In the examples and elsewhere the weight percentages of the ingredients of the solid mixture for making up the bath solution can also be expressed as "parts by weight."

Deposits of varying thicknesses may be plated by the present method, ranging for example from a thickness just sufficient to cover the pores of the basis metal to any practical desired thicker deposit for which a demand may exist.

The invention is useful for articles made of any of a variety of basis metals, such as plain carbon steels, alloy steels including stainless steel, iron, cast iron, copper and copper alloys, nickel and nickel alloys, zinc and zinc alloys, aluminum and aluminum alloys, tin and tin alloys, lead and lead alloys, etc. In general, the basis metal may be any metal, or an undercoat on a metal, that can be chromium plated.

In the light of the foregoing description, the following is claimed:

1. A method of electrodepositing crack-free, chromium plate on a metal article which comprises essentially: pass-

ing current in the range of 0.5 to 8 amperes per square inch from an anode to said article as a cathode immersed in an aqueous chromium plating bath at a temperature of 140° F. to the boiling point of the bath, said bath comprising essentially 300 to 900 g./l. CrO<sub>3</sub>, strontium sulfate and an alkali metal silicofluoride each in an amount sufficient to saturate said bath and to provide therein an undissolved residue of strontium sulfate and alkali metal silicofluoride, respectively, and a soluble non-catalytic alkali metal compound in an amount sufficient to suppress the concentration of the alkali metal silicofluoride in solution in said bath so that the sum of the dissolved sulfate (SO<sub>4</sub><sup>=</sup>) and silicofluoride (SiF<sub>6</sub><sup>=</sup>) is in the range of 2.5 to 10.5 g./l., said alkali metal of the non-catalytic compound being the same as that of the alkali metal silicofluoride and being selected from the group consisting of sodium and potassium, said bath being free of compounds acting to suppress the concentration of dissolved sulfate, and said sum of dissolved sulfate and silicofluoride varying with the CrO<sub>3</sub> concentration in the manner defined by the area ABCD of the graph shown in the accompanying drawing.

2. A method according to claim 1 in which the metal article that is chromium plated is an article of plain carbon steel.

3. A method according to claim 1 in which the temperature of the bath is in the range of 140 to 180° F.

4. A method according to claim 1 in which the alkali metal silicofluoride is potassium silicofluoride and the non-catalytic alkali metal compound is a potassium compound.

5. A method according to claim 1 in which the alkali metal silicofluoride is sodium silicofluoride and the non-catalytic alkali metal compound is a sodium compound.

6. A method of electrodepositing crack-free, chromium plate on a metal article which comprises essentially: passing current in the range of 1 to 3 amperes per square inch from an anode to said article as a cathode immersed in an aqueous chromium plating bath at a temperature of 145 to 160° F., said bath comprising essentially 400 to 900 g./l. CrO<sub>3</sub>, strontium sulfate and an alkali metal silicofluoride each in an amount sufficient to saturate said bath and to provide therein an undissolved residue of strontium sulfate and alkali metal silicofluoride, respectively, and a soluble non-catalytic alkali metal compound in an amount sufficient to suppress the concentration of the alkali metal silicofluoride in solution in said bath so that the sum of the dissolved sulfate and silicofluoride is in the range of 3.0 to 8.5 g./l., said alkali metal of the non-catalytic compound being the same as that of the alkali metal silicofluoride and being selected from the group consisting of sodium and potassium, said bath being free of compounds acting to suppress the concentration of dissolved sulfate, and said sum of dissolved sulfate and silicofluoride varying with the CrO<sub>3</sub> concentration in the manner defined by the area JKLM of the graph shown in the accompanying drawing.

7. An improved method of producing a corrosion resistant chromium plated metal article comprising plating the unplated article, in a single plating operation, in an aqueous bath comprising essentially 300 to 900 g./l. CrO<sub>3</sub>, strontium sulfate and an alkali metal silicofluoride each in an amount sufficient to saturate said bath and to provide therein an undissolved residue of strontium sulfate and alkali metal silicofluoride, respectively, and a soluble non-catalytic alkali metal compound in an amount sufficient to suppress the concentration of the alkali metal silicofluoride in solution in said bath from the unsuppressed saturation concentration of the latter compound to a lower concentration equivalent to 1.0 to 9.0 g./l. of dissolved silicofluoride (SiF<sub>6</sub><sup>=</sup>), the concentration of dissolved sulfate (SO<sub>4</sub><sup>=</sup>) being from 1.5 to 5.5 g./l., the sum of said dissolved sulfate and silicofluoride being in the range of 2.5 to 10.5 g./l., said bath being free of compounds acting to suppress the concentration of dissolved

silicofluoride varying with the CrO<sub>3</sub> concentration in the manner defined by the area JKLM of the graph shown in the accompanying drawing.

sulfate, said sum of dissolved sulfate and silicofluoride varying with the  $\text{CrO}_3$  concentration in the manner defined by the area ABCD of the graph shown in the accompanying drawing, the alkali metal of the non-catalytic compound and of the alkali metal silicofluoride being the same and being selected from the class consisting of potassium and sodium; performing the plating at a bath temperature of 140 to 180° F. and a current density of 0.5

to 8 amperes per square inch; and thereby producing on the article a crack-free deposit of chromium.

References Cited in the file of this patent

UNITED STATES PATENTS

- |           |                |               |
|-----------|----------------|---------------|
| 2,640,021 | Passal         | May 26, 1953  |
| 2,640,022 | Stareck        | May 26, 1953  |
| 2,686,756 | Stareck et al. | Aug. 17, 1954 |